# EUROPEAN PATENT SPECIFICATION

(11) **EP 4 461 838 B1**
(45) Date of publication and mention of the grant of the patent: **18.03.2026**
(21) Application number: 23749474.5
(22) Date of filing: 06.01.2023
(51) Int. Cl.: C22C 38/00, C21D 8/02, C22C 38/14, C22C 38/58, C21D 6/00, C21D 9/46, C22C 38/02, C22C 38/04, C22C 38/08, C22C 38/12, C22C 38/16, C22C 38/22, C22C 38/26, C22C 38/42, C22C 38/46, C22C 38/50

(54) **STEEL PLATE AND METHOD OF PRODUCING SAME**
STAHLPLATTE UND VERFAHREN ZU IHRER HERSTELLUNG
PLATEAU D'ACIER ET SON PROCEDE DE FABRICATION

(30) Priority: 03.02.2022 JP 2022015943
(43) Date of publication of application: 13.11.2024
(73) Proprietor: JFE Steel Corporation, Tokyo 100-0011 (JP)
(72) Inventor: OKUTANI, Masaomi, Tokyo 100-0011 (JP); TERAZAWA, Yusuke, Tokyo 100-0011 (JP); OHTSUBO, Hirofumi, Tokyo 100-0011 (JP)
(74) Representative: Hoffmann Eitle
(86) International application number: PCT/JP2023/000227
(87) International publication number: WO 2023/149157

(56) References cited:
- EP-A1- 2 975 148
- EP-A1- 3 633 057
- WO-A1-2016/035110
- WO-A1-2018/216665
- WO-A1-2021/182618
- JP-A- 2007 302 908
- JP-A- H0 344 417

## Description

### TECHNICAL FIELD

The present invention relates to steel material suitable for steel structures such as ships, marine structures, pressure vessels, line pipes, and offshore wind power generators. In particular, with respect to steel plates having thicknesses exceeding 100 mm, the present invention relates to a thick, high tensile strength steel plate that not only has excellent base metal strength and toughness but also has excellent joint CTOD properties in multilayer fill welded portions, and a method of producing same.

### BACKGROUND

Conventionally, mainly Charpy tests have been used to evaluate steel toughness. In recent years, crack tip opening displacement tests (hereinafter also referred to as CTOD test) have been increasingly applied to steel plates used in steel structures as a method to evaluate fracture resistance with higher precision.

The CTOD test evaluates resistance to occurrence of brittle cracks by introducing a fatigue precrack into a test piece at the location to be evaluated for toughness, subjecting the test piece to three-point bending at low temperature, and measuring the amount of crack opening (plastic deformation) immediately before fracture.

When steel plates are applied to steel structures such as ships, marine structures, pressure vessels, line pipes, wind power generators, and the like, as mentioned above, multilayer fill welding is used. In the multilayer fill weld heat-affected zone (hereinafter also referred to as "multilayer fill weld HAZ"), a zone in the vicinity of the weld line where microstructure has become coarsegrained due to the preceding welding pass (hereinafter also referred to as coarse grain heat-affected zone, or "CGHAZ") is reheated to a two-phase region of ferrite and austenite by a subsequent welding pass, resulting in martensite austenite constituent (hereinafter also referred to as "MA") being mixed into a coarse matrix, resulting in a zone of significantly reduced toughness (hereinafter also referred to as inter-critically reheated coarse grain heat-affected zone, or "ICCGHAZ").

Here, CTOD testing of welded joints is basically performed on the full plate thickness, and therefore when a multilayer fill weld HAZ is the target of evaluation, the region where a fatigue precrack is introduced includes ICCGHAZ microstructure. Further, joint CTOD properties obtained by a joint CTOD test depend on toughness of the most brittle microstructure in the evaluation region, and therefore joint CTOD properties of a multilayer fill weld HAZ reflect the toughness of ICCGHAZ microstructure as well as CGHAZ microstructure.

Therefore, to improve joint CTOD properties of a multilayer fill weld HAZ, it is necessary to improve not only toughness of CGHAZ microstructure but also ICCGHAZ microstructure.

Conventional toughness improvement techniques for the heat-affected zone (HAZ) have been suppression of austenite grain coarsening in the CGHAZ by fine particle distribution of TiN and the use of TiN as a ferrite nucleation site. Here, TiN is sometimes heated to a temperature range where TiN melts in a bonded portion, and therefore when low-temperature toughness requirements for a welded portion are strict, satisfying such requirements has become difficult with only the effect of using TiN.

Further, a technique to suppress austenite grain growth through adding rare earth metals (REM) and dispersing resulting REM acid sulfide, a technique to suppress austenite grain growth through adding Ca and dispersing resulting Ca acid sulfide, and a technique combining the ferrite nucleation capability of BN with oxide dispersion have been used.

For example, Patent Literature (PTL) 1 and PTL 2 describe techniques to suppress austenite grain growth and improve toughness of welded portions by adding REM in combination with Ti and dispersing the fine particles in steel.

Further, PTL 3 proposes a technique for improving toughness of HAZ by using CaS and a technique for improving toughness of base metal by hot rolling.

Further, as a measure for countering toughness decrease at the ICCGHAZ, a technique to increase base metal strength by adding Cu after suppressing the formation of MA by reducing C and Si is proposed in PTL 4.

In addition, in PTL 5, a technique is proposed using BN as a ferrite nucleation site in the heat-affected zone of large-heat input welding to refine HAZ microstructure and improve HAZ toughness.

In recent years, steel structures such as ships, marine structures, pressure vessels, line pipes, and offshore wind power generators have tended to become larger, and steel plates used in steel structures have become thicker and stronger accordingly. Increasing the amount of alloying elements is necessary to achieve steel plates that are both thicker and stronger, but adding large amounts of alloying elements makes securing the toughness of multilayer fill weld HAZ more difficult. To address this problem, PTL 6 describes a technique to improve low-temperature toughness by controlling hardness of a central segregation area.

PTL 7 describes a steel plate comprising a specific chemical composition and having Ceq of 0.45 % or less, where Ceq is defined by the following formula : Ceq (%) = [C] +[Mn] / 6 + ([Cu] + [Ni]) / 15 + ([Cr] + [Mo] + [V]) / 5, and having Pcm of 0.22 % or less, where Pcm is defined by the following formula: Pcm (%) = [C] + [Si] / 30 + ([Mn] + [Cu] + [Cr]) / 20 + [Ni] / 60 + [Mo] / 15 + [V] / 10 + 5 [B], where the brackets indicate a content by mass% of an element enclosed in the brackets and have a value of 0 if such an element is not contained, an average effective grain size of 20 µm or less at a mid-thickness part of the steel plate; and porosities having an equivalent circular diameter of 200 µm or more, the number of the porosities per mm² being 0.1/mm² or less.

PTL 8 describes a steel plate having a composition containing, by mass, C: 0.03% to 0.10%, Si: 0.5% or less, Mn: 1.0% to 2.0%, P: 0.015% or less, S: 0.0005% to 0.0050%, Al: 0.005% to 0.060%, Ni: 0.5% to 2.0%, Ti: 0.005% to 0.030%, N: 0.0015% to 0.0065%, O: 0.0010% to 0.0050%, and Ca: 0.0005% to 0.0060%, with the balance being Fe and inevitable impurities, wherein 1.5 ≤ Ti//N ≤ 5.0, Ceq as defined for PTL 7 is 0.45 or less, Pcm as defined for PTL 7 is 0.20 or less, and 0.2 < (Ca - (0.18 + 130 x Ca) x O) / (1.25 x S) < 1.4, and the effective crystal grain size of the base metal at the center of the steel plate in the thickness direction is 20 µm or less. The densities of a composite inclusion at a 1/4-position and a 1/2-position of the steel plate in a thickness (t: mm) direction, the composite inclusion including a sulfide containing Ca and Mn and an oxide containing Al, the composite inclusion having an equivalent circular diameter of 0.1 µm or more, are each 25 to 250 particle/mm².

### CITATION LIST

### Patent Literature

PTL 1: JP S60-152626 A
PTL 2: JP S60-184663 A
PTL 3: JP 2012-184500 A
PTL 4: JP H05-186823 A
PTL 5: JP S61-253344 A
PTL 6: WO 2014/038200 A1
PTL 7: EP 3 633 057 A1
PTL 8: EP 2 975 148 A1

### SUMMARY

### (Technical Problem)

CTOD specification temperature in standards that specify joint CTOD properties (for example, American Petroleum Institute (API) Recommended Practice RP-2Z) is typically -10 °C.

However, to secure new resources in response to growing energy demand in recent years, the construction range of marine structures and the like has shifted to cold regions and deep-sea regions where resource development has not previously been possible. As a result, there is increasing demand for steel plates that are high-strength, thick-walled, and capable of meeting CTOD specification temperatures that are even lower than those specified by the API standard (for example, -40 °C).

According to investigation by the inventors, the conventional techniques described in PTL 1 to PTL 6 are unable to fully satisfy joint CTOD properties required for multilayer-fill-welded joints for low-temperature specifications in high-strength, thick-walled steel plates having a thickness exceeding 100 mm, which are in high demand in recent years.

For example, PTL 1 and PTL 2 propose techniques for suppressing coarsening of austenite microstructure in the HAZ by adding REM in combination with Ti and dispersing the fine particles in steel. These techniques are intended for steels having relatively low strength and low alloying element content, and therefore cannot be applied to steel material having higher strength and higher alloying element content, because such HAZ microstructure does not include ferrite.

The REM acid sulfide and the Ca acid sulfide in PTL 1 and PTL 2 are effective in inhibiting austenite grain growth. However, the effect of improving toughness by inhibiting austenite grain coarsening of the HAZ cannot alone achieve the joint CTOD properties at the temperatures of low-temperature specifications.

Further, the technique proposed in PTL 3 can satisfy the joint CTOD properties at normal operating temperatures (-10 °C). However, PTL 3 does not consider the joint CTOD properties at the temperatures of low-temperature specifications as described above.

Similarly, PTL 4 does not consider the joint CTOD properties at the temperatures of low-temperature specifications, and it is conceivable that only improving toughness of the ICCGHAZ by decreasing component content of the base metal cannot satisfy low-temperature CTOD specifications. Further, decreasing the alloying element content of the base metal to improve the toughness of the ICCGHAZ is a technical concept that conflicts with securing strength for thicker walls, making it difficult to apply to steel plates used in marine structures and the like.

The technique proposed in PTL 5 is effective when HAZ microstructure is mainly composed of ferrite and a cooling rate of a heat-affected zone is slow, as in large-heat input welding. However, in the case of steel plates exceeding 100 mm in thickness, the amount of alloy components contained in the base metal is relatively high and the heat input in multilayer fill welding is relatively small. Therefore, in multilayer fill welding of steel plates, HAZ microstructure is mainly bainite, and therefore the effect, mentioned above, of improving joint CTOD properties cannot be achieved.

Although PTL 6 proposes a technique for satisfying joint CTOD properties in a low temperature range for steel plates having a thickness of 100 mm or less, equivalent mechanical properties for ultra-thick steel plates having a thickness exceeding 100 mm has not been achieved.

As described above, it is difficult to say that a technique has been established to improve the toughness of the CGHAZ and the ICCGHAZ in the heat-affected zone of multilayer fill welding of high-strength steel plates having a thickness of more than 100 mm. In other words, there was a problem to be solved in improving the CTOD properties of the joint CTOD where a notch position is a bonded portion where the CGHAZ and the ICCGHAZ are mixed.

The present invention has been made in view of the above problems faced by conventional technologies, and it would be helpful to provide a steel plate having a thickness exceeding 100 mm and high strength, as well as excellent CTOD properties at a joint where multilayer fill welding is applied (hereinafter also referred to as multilayer-fill-welded joint CTOD properties), and a method of producing same.

Hereinafter, high strength refers to a yield stress of 320 MPa or more at the mid-thickness position in a tensile test, and excellent multilayer-fill-welded joint CTOD properties refers to a crack opening displacement of 0.30 mm or more at each of a notch position CGHAZ and a sub-critically reheated / inter-critically reheated HAZ (SC/ICHAZ) boundary, at a test temperature of -40 °C.

### (Solution to Problem)

To solve the technical problems described, the inventors have conducted extensive studies to improve joint CTOD properties. As a result, the inventors made the following discoveries.
(1) When pores generated in slab production remain without being closed during rolling, the pores may become defects in the steel plate and become fracture origins. In particular, in order to close pores of a mid-thickness part, it is necessary to appropriately introduce strain into the mid-thickness part during rolling, but this becomes difficult for steel plates having a thickness of more than 100 mm, and therefore remaining pores are a problem. However, the inventors and others have found that when rolling is performed at a high mid-thickness temperature of 950 °C or more, with an average deformation resistance ratio between the mid-thickness part and the surface of a steel plate of 0.70 or less, a rolling reduction ratio of 3 % or more per pass, and a cumulative rolling reduction ratio of 30 % or more, sufficient strain can be introduced into the mid-thickness part, and pores can be sufficiently closed.
   Hereinafter, the mid-thickness part is a region from the center in the thickness direction to a thickness of 10 % of the slab or plate toward both main surfaces of the steel slab or plate.
(2) Further, the mid-thickness part of the slab has element segregation regions, and concentration of alloying elements in these regions causes coarse inclusions to be dispersed at low density. However, as described above, when rolling is performed at a mid-thickness temperature of 950 °C or more, with an average deformation resistance ratio between the mid-thickness part and the surface of the steel plate of 0.70 or less, a rolling reduction ratio of 3 % or more per pass, and a cumulative rolling reduction ratio of 30 % or more, the strain applied to the mid-thickness can be increased. As a result, it was found that coarse inclusions could be elongated and broken up, and fine inclusions could be dispersed to a high density. In addition, as a result of such dispersion, it was found that the HAZ toughness-improving effect of inclusions could be secured.
(3) Further, in order to precipitate and finely disperse TiN in the steel, which is effective in suppressing austenite grain growth, the inventors found that when the composition of the steel plate contains Ti and N satisfying the relationship of 1.50 ≤ Ti/N ≤ 5.00, and, in addition, the equivalent carbon content Ceq is controlled to [C] + [Mn] / 6 + ([Cu] + [Ni]) / 15 + ([Cr] + [Mo] + [V]) / 5 ≤ 0.540 %, and the weld cracking parameter Pcm is controlled to [C] + [Si] / 30 + ([Mn] + [Cu] + [Cr]) / 20 + [Ni] / 60 + [Mo] / 15 + [V] / 10 + 5[B] ≤ 0.250 %, toughness of the matrix of HAZ with multilayer fill welding (hereinafter also referred to as multilayer-fill-welded joint HAZ) can be improved and good joint CTOD properties that can satisfy low-temperature CTOD specifications can be obtained.
   In addition, the inventors and others also studied joint CTOD properties at the sub-critically reheated / inter-critically reheated HAZ (SC/ICHAZ) boundary, which is the boundary between the transformed and untransformed regions of the base metal during welding, as required by the British Standards (BS) EN10225 (2019) and API RP-2Z (2005), which specify the joint CTOD test method. As a result, the inventors made the following discoveries.
(4) In order to satisfy the joint CTOD property requirements at the SC/ICHAZ boundary at a test temperature of -40 °C, the toughness of base metal is dominant over the joint CTOD properties at the SC/ICHAZ boundary, and therefore the inventors found that crystal grain refinement so that the effective crystal grain size of the base metal microstructure is 20 µm or less is required to improve toughness of the base metal.
(5) In steel plates having a thickness exceeding 100 mm, the cooling rate of the mid-thickness part is smaller, resulting in coarsening of the crystal grains at this location. However, the inventors found that by rolling so that the cumulative rolling reduction ratio is 40 % or more under a set of conditions including an average deformation resistance ratio between the mid-thickness part and the surface of the steel plate of 0.70 or less at a mid-thickness temperature of less than 950 °C, sufficient strain can be introduced to the mid-thickness part and crystal grain refinement to the crystal grain size described above can be achieved.

The present invention is based on these findings and further studies. The present invention is defined in the appended claims.

### (Advantageous Effect)

According to the present invention, a steel plate having high strength and excellent multilayer-fill-welded joint CTOD properties may be provided, even when thickness exceeds 100 mm.

### DETAILED DESCRIPTION

The reasons for limitations placed on the features of the present invention are explained below.

### [Chemical composition]

First, the reasons for limiting the chemical composition of the steel plate and the slab to the ranges of the present invention are described. Hereinafter, "%" of each component means mass percentage unless otherwise specified.

### C: 0.02 % to 0.12 %

C is an element that increases hardenability and improves strength of steel. C content needs to be 0.02 % or more. However, the C content exceeding 0.12 % increases the hardness of C-enriched portions and degrades joint CTOD properties. The C content is therefore in the range from 0.02 % to 0.12 %. The lower limit is preferably 0.04 %. The upper limit is preferably 0.09 %.

### Si: 0.70 % or less

Si is an element inevitably contained as an impurity and has an action of improving strength. However, Si content exceeding 0.70 % degrades joint CTOD properties. The Si content is therefore limited to an upper limit of 0.70 %. The upper limit is preferably 0.50 % or less. A lower limit is not particularly limited. The lower limit is preferably about 0.04 %.

### Mn: 0.3 % to 3.0 %

Mn is an element that has the effect of improving strength of the base metal and welded portion through improvement of hardenability of steel. To obtain this effect, addition of 0.3 % or more is required. Mn content is preferably 0.5 % or more. However, addition exceeding 3.0 % not only decreases weldability, but also causes excessive hardenability, which reduces toughness of the base metal and welded portion, resulting in degradation of joint CTOD properties. The Mn content is therefore in the range from 0.3 % to 3.0 %. The Mn content is preferably 2.8 % or less.

### P: 0.050 % or less

P is an element that has a large effect of embrittling grain boundaries, and when added in large amounts decreases HAZ toughness and degrades joint CTOD properties. P content is therefore limited to 0.050 % or less. The P content is preferably 0.030 % or less. Decreasing P content as much as possible is desirable, and therefore a lower limit of the P content is not particularly limited. However, excessively low P content leads to increased refining time and higher costs. The P content is therefore preferably 0.001 % or more.

### S: 0.0050 % or less

S is an element that degrades joint CTOD properties, and therefore an upper limit of S content is limited to 0.0050 %. The upper limit is preferably 0.0030 % or less. Decreasing S content as much as possible is desirable, and therefore a lower limit of the S content is not limited. However, excessively low S content leads to increased refining time and higher costs. The S content is therefore preferably 0.0001 % or more.

### Al: 0.002 % to 0.100 %

Al is an element required for formation of inclusions to improve toughness of multilayer fill weld HAZ and to improve joint CTOD properties, and needs to be added at 0.002 % or more. Al content is preferably 0.005 % or more. However, excessive addition of more than 0.100 % degrades joint CTOD properties in a low temperature range. The Al content is therefore in the range from 0.002 % to 0.100 %. The Al content is preferably 0.075 % or less.

### Ti: 0.002 % to 0.060 %

Ti precipitates in steel as TiN. Precipitated TiN has an effect of inhibiting coarsening of austenite grains in the base metal and HAZ, refining HAZ microstructure and improving joint CTOD properties. To obtain these effects, addition of 0.002 % or more is required. Ti content is preferably 0.005 % or more. However, when the Ti content exceeds 0.060 %, precipitation of solute Ti and coarse TiC decreases toughness of the heat-affected zone and degrades joint CTOD properties. The Ti content is therefore in the range from 0.002 % to 0.060 %. The Ti content is preferably 0.050 % or less.

### N: 0.0130 % or less

N is an element that reduces HAZ toughness and degrades joint CTOD properties, and therefore an upper limit of N content is limited to 0.0130 %. Decreasing N content as much as possible is desirable, and therefore a lower limit of the N content is not limited. However, excessively low N content leads to increased refining time and higher costs. The N content is therefore preferably 0.0005 % or more.

### O: 0.0100 % or less

O is an element that reduces HAZ toughness and degrades joint CTOD properties, and therefore an upper limit of O content is limited to 0.0100 %. Decreasing O content as much as possible is desirable, and therefore a lower limit of the O content is not limited. However, excessively low O content leads to increased refining time and higher costs. The O content is therefore preferably 0.0005 % or more.

The chemical composition of the steel plate according to the present invention consists of the elements described above, optionally including optional elements as described below, with the balance being Fe and inevitable impurity.

According to the present invention, for the purpose of further improving strength, toughness of base metal, joint toughness, and the like, the chemical composition may further optionally contain at least one element selected from the group consisting of Ni, Ca, Cu, Cr, Mo, Nb, V, W, B, REM, and Mg, in a quantity indicated below.

### Ni: 2.0 % or less

Ni is an element that can increase strength of steel plates without significantly degrading toughness of either the base metal or joints, but Ni addition increases production costs and environmental impact. Conventionally, Ni content was required to secure toughness of base metal and joint toughness. However, rolling with a controlled deformation resistance ratio makes it possible to produce high strength steel plates having a thickness of more than 100 mm and excellent multilayer-fill-welded joint CTOD properties without Ni content. On the other hand, Ni may be included to further improve toughness. In such a case, Ni content exceeding 2.0 % increases production costs and environmental impact. The Ni content is therefore limited to 2.0 % or less. The Ni content is more preferably 1.8 % or less. On the other hand, when Ni is added, 0.1 % or more is desirable.

### Ca: 0.0180 % or less

Ca is an element that improves toughness of multilayer fill weld HAZ by forming acid sulfides having high stability at high temperatures, but content exceeding 0.0180 % instead degrades joint CTOD properties. The upper limit of Ca content is therefore limited to 0.0180 %. The Ca content is more preferably 0.0160 % or less. On the other hand, when Ca is added, 0.0002 % or more is desirable.

### Cu: 2.00 % or less

Cu is an element that can increase strength of steel plates without significantly degrading toughness of the base metal and joints. However, when Cu content exceeds 2.00 %, surface cracks caused by a Cu-enriched layer that forms just below scale become a problem. The Cu content is therefore limited to 2.00 % or less. The Cu content is more preferably 1.50 % or less. On the other hand, when Cu is added, 0.05 % or more is desirable.

### Cr: 2.00 % or less

Cr is an element that has an effect of increasing strength of steel through improving hardenability. However, Cr content exceeding 2.00 % degrades joint CTOD properties, and therefore the Cr content is limited to 2.00 % or less. The Cr content is more preferably 1.50 % or less. On the other hand, when Cr is added, 0.05 % or more is desirable.

### Mo: 2.00 % or less

Mo is an element that has an effect of increasing strength of steel through improving hardenability. However, Mo content exceeding 2.00 % degrades joint CTOD properties, and therefore the Mo content is limited to 2.00 % or less. The Mo content is more preferably 1.50 % or less. On the other hand, when Mo is added, 0.05 % or more is desirable.

### Nb: 0.070 % or less

Nb is an element that widens a non-recrystallization temperature range of austenite phase. Therefore, the addition of Nb is effective for efficiently rolling a non-recrystallized region to obtain a fine grain microstructure. When Nb is added, 0.005 % or more is desirable. On the other hand, Nb addition exceeding 0.070 % reduces joint CTOD properties, and therefore Nb content is limited to 0.070 % or less. The Nb content is more preferably 0.050 % or less.

### V: 0.20 % or less

V is an element that improves strength of the base metal, and when V is added, 0.01 % or more is desirable. On the other hand, V content exceeding 0.20 % decreases HAZ toughness and degrades joint CTOD properties, and therefore the V content is limited to 0.20 % or less. The V content is more preferably 0.15 % or less.

### W: 0.50 % or less

W is an element that improves strength of the base metal, and when W is added, 0.05 % or more is desirable. On the other hand, W content exceeding 0.50 % decreases HAZ toughness and degrades joint CTOD properties, and therefore the W content is limited to 0.50 % or less. The W content is more preferably 0.40 % or less.

### B: 0.0050 % or less

B is an element that can improve hardenability and thereby strength of steel plates with only a very small amount of B. When B is added, 0.0005 % or more is desirable. On the other hand, B content exceeding 0.0050 % decreases HAZ toughness and degrades joint CTOD properties, and therefore the B content is limited to 0.0050 % or less. The B content is more preferably 0.0040 % or less.

### REM: 0.030 % or less

Rare earth metals (REM) are elements that inhibit austenite grain growth in the HAZ and improve HAZ toughness by forming acid sulfide inclusions. When REM is added, 0.001 % or more is desirable. On the other hand, REM content exceeding 0.030 % decreases base metal toughness and HAZ toughness and degrades joint CTOD properties. The REM content is therefore limited to 0.030 % or less. The REM content is more preferably 0.025 % or less.

### Mg: 0.0150 % or less

Mg is an element that inhibits growth of austenite grains in the heat-affected zone by forming oxide-based inclusions, improving toughness of the heat-affected zone. When Mg is added, 0.0002 % or more is desirable. On the other hand, when the Mg content exceeds 0.0150 %, the addition effect becomes saturated, and thus an effect commensurate with the content cannot be expected, which becomes economically disadvantageous. The Mg content is therefore limited to 0.0150 % or less. The Mg content is more preferably 0.0100 % or less.

According to the present invention, the chemical composition of the steel plate and the slab is required to further satisfy the Ti/N, Ceq, and Pcm conditions, respectively, as described below. $1 , 50 \leq Ti / N \leq 5,00$

Ti/N controls the amount of solute N and the precipitation state of TiN in the HAZ. When Ti/N is less than 1.50, HAZ toughness degrades due to the presence of solute N that is not fixed as TiN, and joint CTOD properties degrade. On the other hand, when Ti/N is more than 5.00, HAZ toughness degrades due to precipitation of coarse TiN, and joint CTOD properties degrade. The Ti/N range is therefore 1.50 to 5.00. The lower limit is preferably 1.80. The upper limit is preferably 4.50.

### Ceq: 0.280 % or more and 0.540 % or less

When the equivalent carbon content Ceq, defined by the following Expression (2), is increased, microstructure having poor toughness such as martensite austenite constituent and bainite increases in HAZ microstructure, and therefore HAZ toughness degrades. That is, when Ceq is more than 0.540 %, the HAZ matrix itself suffers toughness degradation, and therefore even with HAZ toughness enhancement techniques through inclusions, the required joint CTOD properties cannot be satisfied. On the other hand, when Ceq is less than 0.280 %, the target strength cannot be secured. The Ceq range is therefore 0.280 % to 0.540 %. The lower limit is preferably 0.300 %. The upper limit is preferably 0.500 %. Ceq (%) = [C] + [Mn] / 6 + ([Cu] + [Ni]) / 15 + ([Cr] + [Mo] + [V] / 5

### Pcm: 0.250 % or less

When the weld cracking parameter Pcm defined by the following Expression (3) is increased, microstructure having poor toughness such as martensite austenite constituent and bainite increases in HAZ microstructure, and therefore HAZ toughness degrades. When Pcm exceeds 0.250 %, the HAZ matrix itself suffers toughness degradation, and therefore the required joint CTOD properties cannot be obtained. Pcm is therefore 0.250 % or less. Pcm is preferably 0.240 % or less. A lower limit is not particularly limited, but excessive attempts to reduce Pcm result in too low a Ceq value, and therefore about 0.140 % is preferred. Pcm (%) = [C] + [Si] / 30 + ([Mn] + [Cu] + [Cr]) / 20 + [Ni] / 60 + [Mo] / 15 + [V] / 10 + 5[B]

The square brackets in Expressions (1) to (3) indicate content in mass% of an element enclosed in the brackets and have a value of 0 when the element is not contained.

### [Average effective crystal grain size]

### Average effective crystal grain size at mid-thickness part: 20 µm or less

According to the present invention, average effective crystal grain size of microstructure in the mid-thickness part of the steel plate having a thickness exceeding 100 mm is 20 µm or less. Crystal grains in the mid-thickness part in which segregation is easily caused are refined as described above to improve toughness of the base metal, thereby increasing joint CTOD properties at SC/ICHAZ boundaries. The smaller the average effective crystal grain size, the more advantageous, and therefore the average effective crystal grain size is not particularly limited. Typically, a lower limit is about 1 µm.

Here, "effective crystal grain size" is defined as the circle equivalent diameter of a crystal grain surrounded by grain boundaries of crystal grains having an orientation difference of 15° or more, that is, large-angle grain boundaries. Further, the average effective crystal grain size in the mid-thickness part can be measured by a method described in the following EXAMPLES section.

### [Pore number density]

### Pore number density: 0.10/mm² or less

As mentioned above, residual pores in the steel plates become fracture origins, which degrade joint CTOD properties. In particular, when the number of pores having a circle equivalent diameter of 180 µm or more per mm² (hereinafter also referred to simply as "pore number density") in the steel plate exceeds 0.10, the possibility of insufficient crack opening displacement (δ) in the joint CTOD test becomes extremely high. Further, as the pore number density increases, the yield stress at the mid-thickness part of the base material decreases. Accordingly, limiting the pore number density to 0.10/mm² or less is important.

Hereinafter, the pore number density means an average number density across full thickness × full width in a cross-section parallel to the transverse direction of a steel plate (cross section perpendicular to the rolling direction). The pore number density may be measured by the method described in the EXAMPLES section below, but the measurement method is not limited to the method described in the EXAMPLES section and any known measurement method may be used for measurement.

Further, measurement frequency of the pore number density may be measuring one or two cross-sections of any one steel plate among steel plates prepared from steel slabs under the same steelmaking and rolling conditions. As long as the slab steelmaking method and rolling conditions are not changed, the pore number density is highly reproducible, and therefore measurement results at the above measurement frequency are representative of the whole.

### [Production method]

Next, the reasons for limiting each condition in the method of producing the steel plate according to the present invention are explained below. In the following description, "temperature" means temperature at the mid-thickness part, unless otherwise noted. Temperature at the mid-thickness part may be measured as described in the following EXAMPLES section. However, for example, on an actual production line, temperature at a surface of a steel plate may be measured using a radiation thermometer and temperature at the mid-thickness part may be determined by heat transfer calculation.

### • Slab heating conditions

According to the present invention, a method of preparing the slab is not particularly limited, and any known steelmaking method may be applied, such as a converter, an electric furnace, a vacuum melting furnace, and the like. The slab may be produced, for example, by a continuous casting method. Further, molten steel from which the slab is produced may be further subjected to secondary refining such as ladle refining.

The slab produced as described above is heated to a temperature of 990 °C or more and 1200 °C or less. When the heating temperature is lower than 990 °C, the following conditions of hot rolling cannot be met, and a sufficient effect cannot be obtained. On the other hand, when the heating temperature is higher than 1200 °C, austenite grains become coarse and the desired fine grain microstructure cannot be obtained after controlled rolling. For these reasons, the range of the heating temperature is 990 °C or more to 1200 °C or less. The lower limit of temperature is preferably 990 °C, and the upper limit of temperature is preferably 1180 °C.

### • Hot rolling conditions

During the hot rolling, it is important to control hot rolling conditions in both a recrystallization temperature range and a non-recrystallization temperature range.

In the recrystallization temperature range, rolling is performed at 950 °C or more, the rolling reduction ratio is 3 % or more per pass, and the cumulative rolling reduction ratio is 30 % or more, under a set of conditions including the average deformation resistance ratio between the mid-thickness part and the surface of the steel plate being 0.70 or less.

### [Deformation resistance ratio between mid-thickness part and surface of steel plate: 0.70 or less]

According to the present invention, the average value of the ratio of the deformation resistance k_{fm} (mid-thickness) of the mid-thickness part to the deformation resistance k_{fm} (surface) of the surface of the steel plate, as defined by the following Expressions (5) to (7), is 0.70 or less (Expression (4)). Specifically, the average deformation resistance ratio between the mid-thickness part and the surface made to be 0.70 or less by rolling at the timing when the temperature difference between mid-thickness and surface is at an appropriate value according to the mass% of C, while adjusting roller rotational speed, roller radius, and roll gap to appropriate values. ${k}_{fm} \left(mid-thickness\right) / {k}_{fm} \left(surface\right) \leq 0.70$ (Here, k_{fm} is derived from Expression (5))
[Math. 1] ${k}_{fm} = {e}^{\left(0.126-1.75\left[C\right]+0.594{\left[C\right]}^{2}+\frac{2851 + 2968 \left[C\right] - 1120 {\left[C\right]}^{2}}{{T}_{k}}\right)} \times {ε}^{0.21} \times {\dot{ε}}^{0.13}$ where *ε* is derived from Expression (6) and *ε̇* is derived from Expression (7)
[Math. 2] $ε = ln \frac{{h}_{1}}{{h}_{0}}$
[Math. 3] $\dot{ε} = \frac{2 πn}{60 \sqrt{r}} \times \sqrt{\frac{R}{{h}_{0}}} \times ln \left(\frac{1}{1 - r}\right)$

In Expressions (5) to (7), [C] is mass% of C, Tₖ is absolute temperature (K) at the point where k_{fm} is determined, that is, the mid-thickness or steel plate surface, h₀ is thickness on rolling entry, h₁ is thickness on rolling delivery, n is the roller rotational speed (rpm), r is rolling reduction, and R is roller radius (mm).

Temperature at the surface may be measured by a radiation thermometer, and temperature at the mid-thickness part may be measured as described in the following EXAMPLES section. However, for example, on an actual production line, temperature at a surface of a steel plate may be measured using a radiation thermometer and temperature at the mid-thickness part may be determined by heat transfer calculation.

Under conditions where the average value of the deformation resistance ratio between the mid-thickness part and the surface of a steel plate according to Expression (4) exceeds 0.70, sufficient strain cannot be introduced into the mid-thickness part of a steel plate having a thickness exceeding 100 mm, and pores will remain. As a result, the pore number density cannot be made to be 0.10/mm² or less. Therefore, the ratio of deformation resistance between the mid-thickness part and the surface of the steel plate is 0.70 or less, the rolling reduction ratio is 3 % or more per pass, and the cumulative rolling reduction ratio is 30 % or more.

### [Rolling at 950 °C or more]

A purpose of rolling at 950 °C or more is to close pores in addition to refining microstructure by recrystallization and refining and dispersing coarse inclusions. That is, rolling at less than 950 °C makes it difficult for recrystallization to occur, resulting in insufficient refinement of austenite grains.

### [Rolling reduction ratio of 3 % or more per pass]

Rolling with a reduction ratio of less than 3 % per pass does not introduce sufficient strain in the mid-thickness part, and even when rolling reduction ratio is 3 % or more per pass, a cumulative rolling reduction ratio of less than 30 % does not sufficiently close pores.

### [Rolling at less than 950 °C]

In rolling at the non-recrystallization temperature range, that is, less than 950 °C, the cumulative rolling reduction ratio is 40 % or more, under the same condition of the average deformation resistance ratio between the mid-thickness part and the surface of the steel plate being 0.70 or less.

The steel according to the present invention is difficult to recrystallize when rolled at temperatures less than 950 °C, and therefore the strain introduced by rolling is not consumed by recrystallization but accumulates and acts as nucleation sites in the subsequent cooling process. As a result, the finally obtained steel plate can have a refined microstructure. However, the crystal grain refinement effect is insufficient under conditions where the cumulative rolling reduction ratio in this temperature range is less than 40 %. Further, in a steel plate having a thickness exceeding 100 mm, under a set of conditions where the average deformation resistance ratio between the mid-thickness part and the surface of the steel plate exceeds 0.70, sufficient strain cannot be introduced into the mid-thickness part, the refinement of the final microstructure in the mid-thickness part becomes insufficient, and the average effective crystal grain size in the mid-thickness part cannot be 20 µm or less.

Therefore, rolling at the non-recrystallization temperature range has a cumulative rolling reduction ratio of 40 % or more, and the average deformation resistance ratio between the mid-thickness part and the surface of the steel plate is 0.70 or less.

### [Cooling]

After completion of the hot rolling, the obtained hot-rolled steel plate is cooled. The cooling can be performed by any method as long as the following conditions are met. For example, the cooling may be performed by water cooling.

### Average cooling rate: 1.0 °C/s or more

When the average cooling rate at the mid-thickness temperature is less than 1.0 °C/s, coarse ferrite phase occurs in the base metal microstructure, and therefore joint CTOD properties of the SC/ICHAZ degrade. The average cooling rate at the mid-thickness position is therefore 1.0 °C/s or more. On the other hand, when the average cooling rate is greater than 50.0 °C/s, an increase in hard bainite phase increases strength of the base metal and degrades joint CTOD properties of the SC/ICHAZ, and therefore the cooling rate is preferably 50.0 °C/s or less.

According to the present invention, when the cooling stop temperature indicated in the next paragraph is 500 °C or less, the average value from 700 °C to 500 °C is the average cooling rate described above, and when the cooling stop temperature is higher than 500 °C, the average value from 700 °C to the cooling stop temperature higher than 500 °C is the average cooling rate described above.

### Cooling stop temperature: 600 °C or less

In the cooling, the hot-rolled steel plate is cooled to a cooling stop temperature that is 600 °C or less at mid-thickness temperature. When the cooling stop temperature is higher than 600 °C, microstructure after transformation becomes coarse, resulting in insufficient base metal strength and degradation of SC/ICHAZ joint CTOD properties. The cooling stop temperature is therefore 600 °C or less.

### [Tempering treatment]

### Tempering Temperature: 700 °C or less

After the cooling stop, the steel plate may be subjected to tempering treatment. Tempering treatment can further improve the toughness of base metal. At this time, a tempering temperature higher than 700 °C generates a coarse ferrite phase, thus degrading toughness of the SCHAZ. The tempering temperature is therefore preferably 700 °C or less. The tempering temperature is more preferably 650 °C or less. A lower limit of the tempering temperature is not particularly limited. The lower limit may be about 300 °C.

In the method of production according to the present invention, anything not described herein may follow a conventional method.

### EXAMPLES

More detailed description is given below based on examples. The following examples merely represent preferred examples, and the present invention is not limited to these examples.

Slabs having a chemical composition listed in Table 1 were used to produce steel plates under the production conditions listed in Table 2. During hot rolling, a thermocouple was attached in a central position in the longitudinal direction, width direction, and thickness direction of each steel material to be hot rolled to measure the temperature of the mid-thickness part. At the same time, surface temperature of the steel material was measured with a radiation thermometer.

The average effective crystal grain size, the pore number density, and the yield stress of each obtained steel plate were measured by the following methods.

### [Average effective crystal grain size]

A sample was collected from each obtained steel plate so that a measurement position was located at a central position in the longitudinal direction, width direction, and thickness direction of the steel plate. Then, after mirror polishing a surface of the sample, electron backscatter pattern (EBSP) analysis was performed under the following conditions. From an obtained crystal orientation map, a circle equivalent diameter of a microstructure surrounded by a large-angle grain boundary having an orientation difference of 15° or more from adjacent crystal grains was determined, and an average of the circle equivalent diameters in the following analysis region was defined as an average effective crystal grain size.

### EBSP Conditions

- Analysis region: 1 mm × 1 mm area at mid-thickness
- Step size: 0.4 µm

### [Pore number density]

For detection of defects inside of a steel plate, ultrasonic testing is often used because ultrasonic testing can perform nondestructive inspection. However, to precisely check the state of defects, the inside of the steel plates were directly observed to measure the pore number density. First, a sample was taken in a thickness direction cross-section parallel to the plate transverse direction (cross-section perpendicular to the rolling direction) of the rolled material from a central position of the plate length, for observation where the observation plane is the full thickness × full width size, and finished with mirror polishing. Next, the mirror-polished sample was observed using an optical microscope and image captured. The obtained images were subjected to image analysis to determine the circle equivalent diameter of each pore found in the image. The number of pores having a size of 180 µm or more was divided by the measured area (plate thickness × plate width) to determine the number of pores having a circle equivalent diameter of 180 µm or more per mm².

### [Yield stress]

Tensile tests were conducted according to EN 10002-1 to determine yield stress (YS) at 1/4 and 1/2 positions of thickness (t) of each steel plate. For each tensile test, a round bar tensile test piece having a parallel portion diameter of 14 mm and a parallel portion length of 70 mm was used, the test pieces being taken parallel to the plate transverse direction from 1/4 and 1/2 positions of plate thickness. In the tensile test, when an upper yield point appeared, the upper yield point was determined to be yield stress. Further, when an upper yield point did not appear, a 0.2 % proof stress was determined to be yield stress.

Next, each steel plate was used to produce a multilayer-fill-welded joint. Each obtained multilayer-fill-welded joint was subjected to a joint CTOD test to measure the amount of crack opening displacement in the CGHAZ and the amount of crack opening displacement in the SC/ICHAZ. The conditions for production of the multilayer-fill-welded joints and the conditions of the joint CTOD tests are described below.

### [Joint CTOD test]

Welded joints used for the joint CTOD tests were produced by submerged arc welding (multilayer fill welding) with K groove geometry and heat input of 5.0 kJ/mm. The test method was based on BS EN10225 (2019), and the crack opening displacement [CTOD value (δ)] was evaluated at the test temperature of -40 °C using test pieces each having a square cross-section of t × t (where t is plate thickness).

In the joint CTOD tests described above, a test where the notch position was set as the CGHAZ on the linear side of the K groove and a test where the notch position was set at the SC/ICHAZ boundary were conducted, and the δ of the CGHAZ and the δ of the SC/ICHAZ boundary were measured, respectively. For each steel plate, the test was performed for three test pieces per notch position and the lowest value measured was taken as δ.

After the tests, on a fracture surface of the test piece, the end of a fatigue precrack was confirmed to be located both in the CGHAZ and at the SC/ICHAZ boundary specified by EN10225 (2019). In the case of joint CTOD test of multilayer fill welding, even when a notch position is located in the CGHAZ, a certain amount of the ICCGHAZ is also included, and therefore the test result reflects toughness of both the CGHAZ and the ICCGHAZ.

The measurement results are listed in Table 2.

As can be seen in Table 2, the steel plates satisfying the conditions of the present invention (Examples) had manufacturing conditions, effective crystal grain size of the base metal, and pore number densities all within acceptable ranges, yield stress at the 1/4 thickness position and at the mid-thickness position of 320 MPa or more, CTOD values at the CGHAZ and CTOD values at the SC/ICHAZ boundary both 0.30 mm or more at -40 °C, and combined high strength with excellent joint CTOD properties.

In contrast, among the steel plates that did not satisfy the conditions of the present invention (Comparative Examples), No. 42, No. 43, and No. 47 each had a yield stress of less than 320 MPa at the 1/4 thickness position and at the mid-thickness position. No. 20 had a yield stress of less than 320 MPa at the 1/4 thickness position and at the mid-thickness position and a CTOD value of less than 0.30 mm at the SC/ICHAZ boundary. No. 52 had a yield strength of 320 MPa or more at the 1/4 thickness position, but the yield stress at the mid-thickness position was less than 320 MPa. Other Comparative Examples had one or both of the CTOD values of the CGHAZ and the SC/ICHAZ boundary less than 0.30 mm. All of the Comparative Examples had inferior base metal strength and joint CTOD properties compared to the Examples.

## Claims

1. A steel plate having a thickness exceeding 100 mm and a yield stress of 320 MPa or more and comprising a chemical composition containing, in mass%,
C: 0.02 % to 0.12 %,
Si: 0.70 % or less,
Mn: 0.3 % to 3.0 %,
P: 0.050 % or less,
S: 0.0050 % or less,
Al: 0.002 % to 0.100 %,
Ti: 0.002 % to 0.060 %,
N: 0.0130 % or less,
O: 0.0100 % or less, and
optionally at least one selected from the group consisting of
Ni: 2.0 % or less,
Ca: 0.0180 % or less,
Cu: 2.00 % or less,
Cr: 2.00 % or less,
Mo: 2.00 % or less,
Nb: 0.070 % or less,
V: 0.20 % or less,
W: 0.50 % or less,
B: 0.0050 % or less,
REM: 0.030% or less and,
Mg: 0.0150 % or less,
with the balance being Fe and inevitable impurity, wherein the chemical composition satisfies Expressions (1) to (3) below, and
the average effective crystal grain size in a mid-thickness part is 20 µm or less, and the number of pores in the steel plate having a circle equivalent diameter of 180 µm or more is 0.10 or less per mm²,
wherein
the yield strength is determined at the mid-thickness position in a tensile test as described in the description,
the effective crystal grain size is defined as the circle equivalent diameter of a crystal grain surrounded by grain boundaries of crystal grains having an orientation difference of 15° or more,
the average effective crystal grain size in a mid-thickness part is determined by a method as described in the description, and
the number of pores in the steel plate is the pore number density and is determined by a method as described in the description, $1.50 \leq Ti / N \leq 5.00$ 0.280 % ≤ Ceq (= [C] + [Mn] / 6 + ([Cu] + [Ni]) / 15 + ([Cr] + [Mo] + [V]) / 5) ≤ 0.540 % Pcm (= [C] + [Si] / 30 + ([Mn] + [Cu] + [Cr]) / 20 + [Ni] / 60 + [Mo] / 15 + [V] / 10 + 5[B]) ≤ 0.250 %
where the square brackets in Expressions (1) to (3) indicate content in mass% of an element enclosed in the brackets and have a value of 0 when the element is not contained.

2. A method of producing the steel plate according to claim 1, the method comprising:
heating a slab having the chemical composition according to claim 1 to a temperature range from 990 °C or more to 1200 °C or less; hot rolling the under a set of conditions satisfying Expression (4) below, with a mid-thickness temperature of 950 °C or more, a rolling reduction ratio of 3 % or more per pass, and a cumulative rolling reduction ratio of 30 % or more; hot rolling at a mid-thickness temperature of less than 950 °C and a cumulative rolling reduction ratio of 40 % or more; then, when cooling to a cooling stop temperature of 600 °C or less at an average cooling rate at mid-thickness of 1.0 °C/s or more, when the cooling stop temperature is 500 °C or less, the average value from 700 °C to 500 °C is the average cooling rate, and when the cooling stop temperature is higher than 500 °C, the average value from 700 °C to the cooling stop temperature that is higher than 500 °C is the average cooling rate,
wherein the mid-thickness temperature is measured as described in the description, ${k}_{fm} \left(mid-thickness\right) / {k}_{fm} \left(surface\right) \leq 0.70$
where k_{fm} is derived from Expression (5),
[Math. 1] ${k}_{fm} = {e}^{\left(0.126-1.75\left[C\right]+0.594{\left[C\right]}^{2}+\frac{2851 + 2968 \left[C\right] - 1120 {\left[C\right]}^{2}}{{T}_{k}}\right)} \times {ε}^{0.21} \times {\dot{ε}}^{0.13}$ where ε is derived from Expression (6) and ε̇ is derived from Expression (7)
[Math. 2] $ε = ln \frac{{h}_{1}}{{h}_{0}}$ [Math. 3] $\dot{ε} = \frac{2 πn}{60 \sqrt{r}} \times \sqrt{\frac{R}{{h}_{0}}} \times ln \left(\frac{1}{1 - r}\right)$
where, in Expressions (5) to (7), [C] is mass% of C, Tₖ is absolute temperature in K at mid-thickness or steel plate surface, h₀ is thickness on rolling entry, h₁ is thickness on rolling delivery, n is the roller rotational speed in rpm, r is rolling reduction, and R is roller radius in mm.

3. The method of producing a steel plate according to claim 2, wherein, after the cooling to the cooling stop temperature, a tempering treatment is performed at a temperature of 700 °C or less.

## Patentansprüche

1. Stahlplatte mit einer Dicke über 100 mm und einer Streckgrenze von 320 MPa oder mehr und umfassend eine chemische Zusammensetzung, enthaltend in Masse-%
C: 0,02 % bis 0,12 %,
Si: 0,70 % oder weniger,
Mn: 0,3 % bis 3,0 %,
P: 0,050 % oder weniger,
S: 0,0050 % oder weniger,
Al: 0,002 % bis 0,100 %,
Ti: 0,002 % bis 0,060 %,
N: 0,0130 % oder weniger,
O: 0,0100 % oder weniger und
optional mindestens eines, ausgewählt aus der Gruppe, bestehend aus
Ni: 2,0 % oder weniger,
Ca: 0,0180 % oder weniger,
Cu: 2,00 % oder weniger,
Cr: 2,00 % oder weniger,
Mo: 2,00 % oder weniger,
Nb: 0,070 % oder weniger,
V: 0,20 % oder weniger,
W: 0,50 % oder weniger,
B: 0,0050 % oder weniger,
REM: 0,030 % oder weniger und
Mg: 0,0150 % oder weniger,
wobei der Rest Fe und unvermeidliche Verunreinigungen ist, wobei die chemische Zusammensetzung die nachstehenden Ausdrücke (1) bis (3) erfüllt und
die durchschnittliche effektive Kristallkorngröße in einem Abschnitt in der Mitte der Dicke 20 µm oder weniger beträgt und die Anzahl an Poren in der Stahlplatte mit einem äquivalenten Kreisdurchmesser von 180 µm oder mehr 0,10 oder weniger pro mm² beträgt,
wobei
die Streckgrenze an der Position in der Mitte der Dicke in einem Zugversuch wie in der Beschreibung beschrieben bestimmt wird,
die effektive Kristallkorngröße als äquivalenter Kreisdurchmesser eines Kristallkorns definiert ist, das durch Korngrenzen von Kristallkörnern mit einem Orientierungsunterschied von 15° oder mehr umgeben ist,
die durchschnittliche effektive Kristallkorngröße in einem Abschnitt in der Mitte der Dicke durch ein in der Beschreibung beschriebenes Verfahren bestimmt wird und
die Anzahl der Poren in der Stahlplatte die Porenzahldichte ist und durch ein in der Beschreibung beschriebenes Verfahren bestimmt wird, $1 , 50 \leq Ti / N \leq 5 , 00$ 0,280 % ≤ Ceq (=[C] + [Mn]/6 + ([Cu] + [Ni])/15 + ([Cr] + [Mo] + [V])/5) ≤ 0,540 % Pcm (=[C] + [Si]/30 + ([Mn] + [Cu]+ [Cr])/20 + [Ni]/60 + [Mo]/15 + [V]/10 + 5[B]) ≤ 0,250 %
wobei die eckigen Klammern in den Ausdrücken (1) bis (3) einen Gehalt in Masse-% eines in den Klammern eingeschlossenen Elements angeben und einen Wert von 0 aufweisen, wenn das Element nicht enthalten ist.

2. Verfahren zur Herstellung der Stahlplatte gemäß Anspruch 1, wobei das Verfahren umfasst:
Erwärmen einer Bramme mit der chemischen Zusammensetzung gemäß Anspruch 1 auf einen Temperaturbereich von 990°C oder mehr bis 1.200°C oder weniger, Warmwalzen dieser unter Bedingungen, die den nachstehenden Ausdruck (4) erfüllen, bei einer Temperatur in der Mitte der Dicke von 950°C oder mehr, einem Walzreduktionsgrad von 3 % oder mehr pro Walzstich und einem kumulativen Walzreduktionsgrad von 30 % oder mehr, Warmwalzen bei einer Temperatur in der Mitte der Dicke von weniger als 950°C und einem kumulativen Walzreduktionsgrad von 40 % oder mehr, anschließend beim Abkühlen auf eine Abkühlungsstopptemperatur von 600°C oder weniger bei einer durchschnittlichen Abkühlungsgeschwindigkeit in der Mitte der Dicke von 1,0°C/s oder mehr, wenn die Abkühlungsstopptemperatur 500°C oder weniger beträgt, der Durchschnittswert von 700°C bis 500°C die durchschnittliche Abkühlungsgeschwindigkeit ist, und wenn die Abkühlungsstopptemperatur höher als 500°C ist, der Durchschnittswert von 700°C bis zur Abkühlungsstopptemperatur, die höher als 500°C ist, die durchschnittliche Abkühlungsgeschwindigkeit ist,
wobei die Temperatur in der Mitte der Dicke wie in der Beschreibung beschrieben gemessen wird, ${k}_{fm} \left(Mitte der Dicke\right) / \left({k}_{fm}\left(Oberfläche\right)\right. \leq 0 , 70$
worin k_{fm} aus dem Ausdruck (5) abgeleitet wird,
[Math. 1] ${k}_{fm} = {e}^{\left(0. 126-1. 75\left[C\right]+0. 594{\left[C\right]}^{2}+\frac{2851 + 2968 \left[C\right] - 1120 {\left[C\right]}^{2}}{{T}_{k}}\right)} \times {ε}^{0 . 21} \times {\dot{ε}}^{0 . 13}$
worin ε aus dem Ausdruck (6) abgeleitet wird und ε̇ aus dem Ausdruck (7) abgeleitet wird
[Math 2] $ε = ln \frac{h 1}{{h}_{0}}$ [Math. 3] $\dot{ε} = \frac{2 πn}{60 \sqrt{r}} \times \sqrt{\frac{R}{{h}_{0}}} \times ln \left(\frac{1}{1 - r}\right)$
wobei in den Ausdrücken (5) bis (7) [C] Masse-% von C ist, Tₖ eine absolute Temperatur in K in der Mitte der Dicke oder der Stahlplattenoberfläche ist, h₀ eine Dicke beim Walzeintritt ist, h₁ eine Dicke beim Walzaustritt ist, n die Walzenrotationsgeschwindigkeit in U/min ist, r die Walzreduktion ist und R der Walzenradius in mm ist.

3. Verfahren zur Herstellung einer Stahlplatte gemäß Anspruch 2, wobei nach dem Abkühlen auf die Abkühlungsstopptemperatur eine Anlassbehandlung bei einer Temperatur von 700°C oder weniger durchgeführt wird.

## Revendications

1. Tôle d'acier présentant une épaisseur dépassant 100 mm et une limité de contrainte de 320 MPa ou plus et comprenant une composition chimique contenant, en % en masse,
C : 0,02 % à 0,12 %,
Si : 0,70 % ou moins,
Mn : 0,3 % à 3,0 %
P : 0,050 % ou moins,
S : 0,0050 % ou moins,
Al : 0,002 % à 0,100 %,
Ti : 0,002 % à 0,060 %,
N : 0,0130 % ou moins,
O : 0,0100 % ou moins, et
optionnellement au moins un sélectionné parmi le groupe constitué de Ni : 2,0 % ou moins,
Ca : 0,0180 % ou moins,
Cu : 2,00 % ou moins,
Cr : 2,00 % ou moins,
Mo : 2,00 % ou moins,
Nb : 0,070 % ou moins,
V : 0,20 % ou moins,
W : 0,50 % ou moins,
B : 0,0050 % ou moins,
REM : 0,030 % ou moins et,
Mg : 0,0150 % ou moins,
avec le reste étant Fe et une impureté inévitable, dans lequel la composition chimique satisfait aux expressions (1) à (3) ci-dessous, et
la taille moyenne effective de grain cristallin dans une partie de mi-épaisseur est de 20 µm ou moins, et le nombre de pores dans la tôle d'acier présentant un diamètre équivalent circulaire de 180 µm ou plus est 0,10 ou moins par mm²,
dans lequel
la résistance à la déformation est déterminée à la position de mi-épaisseur lors d'un essai de traction comme décrit dans la description,
la taille effective de grain cristallin est définie comme le diamètre équivalent du cercle d'un grain cristallin entouré de limites de grains de grains cristallins présentant une différence d'orientation de 15° ou plus,
la taille moyenne effective de grain cristallin dans une partie de mi-épaisseur est déterminée par un procédé tel que décrit dans la description, et
le nombre de pores dans la tôle d'acier est la densité de nombre de pores et est déterminé par un procédé tel que décrit dans la description, $1 , 50 \leq Ti / N \leq 5,00$ 0,280 % ≤ Ceq (= [C] + [Mn]/ 6 + ([Cu] + [Ni]) /15 + ([Cr] + [Mo] + [V]) /5) ≤ 0,540 % ...(2) Pcm (= [C] + [Si] /30 + ([Mn] + [Cu] + [Cr]) /20 + [Ni] /60 + [Mo] /15 + [V] /10 + 5[B]) ≤ 0,250 % ...(3)
où les crochets dans les expressions (1) à (3) indiquent le contenu en % en masse d'un élément enfermé dans les crochets et présentent une valeur de 0 lorsque l'élément n'est pas contenu.

2. Procédé de production de la tôle d'acier selon la revendication 1, le procédé comprenant :
le chauffage d'une brame présentant la composition chimique selon la revendication 1 à une plage de température allant de 990 °C ou plus à 1 200 °C ou moins ; laminage à chaud sous un ensemble de conditions satisfaisant à l'expression (4) ci-dessous, avec une température de mi-épaisseur de 950 °C ou plus, un taux de réduction de laminage de 3 % ou plus par passe, et un taux de réduction de laminage cumulatif de 30 % ou plus ; laminage à chaud à une température de mi-épaisseur inférieure à 950 °C et un taux de réduction de laminage cumulatif de 40 % ou plus ; alors, lors du refroidissement à une température d'arrêt de refroidissement de 600 °C ou moins à un taux de refroidissement moyen à mi-épaisseur de 1,0 °C/s ou plus, lorsque la température d'arrêt de refroidissement est de 500°C ou moins, la valeur moyenne de 700 °C à 500°C est le taux de refroidissement moyen, et lorsque la température d'arrêt de refroidissement est supérieure à 500 °C, la valeur moyenne de 700 °C à la température d'arrêt de refroidissement qui est supérieure à 500 °C est le taux de refroidissement moyen,
dans lequel la température de mi-épaisseur est mesurée tel que décrit dans la description, ${k}_{fm} \left(mi-épaisseur\right) / {k}_{fm} \left(surface\right) \leq 0 , 70$ où k_{fm} est dérivé de l'expression (5), ${k}_{fm} = {e}^{\left(0.126-1.75\left[C\right]+0.594{\left[C\right]}^{2}+\frac{2851 + 2968 \left[C\right] - 1120 {\left[C\right]}^{2}}{{T}_{k}}\right)} \times {ε}^{0.21} \times {\dot{ε}}^{0.13}$ où ε est dérivé de l'expression (6) et έ est dérivé de l'expression (7)
[Math. 2] $ε = ln \frac{{h}_{1}}{{h}_{0}}$
[Math. 3] $\dot{ε} = \frac{2 πn}{60 \sqrt{r}} \times \sqrt{\frac{R}{{h}_{0}}} \times ln \left(\frac{1}{1 - r}\right)$
où, dans les expressions (5) à (7), [C] est le % en masse de C, Tₖ est une température
absolue dans K
à mi-épaisseur ou une surface de la tôle d'acier, h₀ est l'épaisseur à l'entrée du laminage, h₁ est l'épaisseur à la sortie du laminage, n est la vitesse de rotation du rouleau en tr/min, r est la réduction de laminage, et R est le rayon du rouleau en mm.

3. Procédé de production d'une tôle d'acier selon la revendication 2, dans lequel, après le refroidissement jusqu'à la température d'arrêt de refroidissement, un traitement de revenu est réalisé à une température de 700 °C ou moins.
